

# UNITED STATES PATENT OFFICE.

HUGH C. SICARD, OF BUFFALO, NEW YORK, ASSIGNOR TO UNITED STATES FERRO-  
ALLOYS CORPORATION, OF NEW YORK, N. Y., A CORPORATION OF NEW YORK.

## PROCESS FOR PRODUCTION OF LOW-CARBON FERROCHROME.

1,341,939.

Specification of Letters Patent. Patented June 1, 1920.

No Drawing.

Application filed September 26, 1919. Serial No. 326,646.

*To all whom it may concern:*

Be it known that I, HUGH C. SICARD, a citizen of the United States of America, and a resident of the city of Buffalo, county of Erie, and State of New York, have invented a new and useful Process for the Production of Low-Carbon Ferrochrome, of which the following is a full, clear, and exact description.

10 This invention relates generally to a method of manufacturing and producing low carbon ferrochrome.

In another co-pending patent application, identified as Serial No. 318,331, filed August 15 18, 1919, I have described a method of making an alloy of iron, chromium and titanium, having a variable carbon content, the carbon of which is present as a carbid or carbids of iron, chromium and titanium.

20 It has been a common practice of the art in decarbonizing ferro-chrome to use chrome ore, such as chromite, in combination with burnt lime, of which the latter forms a protective blanket of slag over the molten metal. The chrome ore then reacts with the ferro-chrome which contains carbon, and thus in time becomes decarbonized. When such methods are used, the iron oxid which is present in the chrome ore is more 30 readily reduced than the oxid of chromium, and the consequence is that when the final decarbonized ferro-chrome is obtained, it is found to have a lower content of chromium than the original high carbon material.

35 In producing this invention I have overcome the difficulties above referred to.

In carrying out my invention I use titanic oxid ( $TiO_2$ ) for the purpose of decarbonization. This oxid reacts with the carbon in 40 the high carbon ferro-chrome and forms titanium according to the following equation:



It is important to use as a source of the 45 titanic oxid some ore which contains the least possible amount of iron oxid, such as rutile.

The reaction is carried out in an electric furnace of the well-known Heroult type, for 50 example. In this furnace is charged a mixture of the alloy of ferro-chromium, which

is high in carbon and a quantity of rutile which will be sufficient to decarbonize the alloy used. In place of the ferro-chromium I may use an alloy of iron chromium and 55 titanium, which is high in carbon. Into this charge burnt lime is placed and the charge is melted down. The burnt lime forms a protective slag and when the reaction is complete the resulting alloy is tapped from 60 the furnace.

Having thus described my invention, what I claim is:

1. The method of making low carbon alloys of iron, chromium and titanium 65 which consists in the decarbonization of a high carbon ferro-chromium alloy by means of titanic oxid.

2. The method of making low carbon alloys of iron, chromium and titanium 70 which consists in the decarbonization of a high carbon ferro-chromium alloy by means of an ore high in titanic oxid and low in iron oxid.

3. The method of making low carbon 75 alloys of iron, chromium and titanium, which consists in the decarbonization of a high carbon ferro-chromium alloy by means of rutile ore.

4. The method of making low carbon 80 alloys of iron, chromium and titanium, which consists in charging into an electric furnace a mixture of ferro-chromium high in carbon, and a sufficient quantity of titanic oxid to decarbonize the alloy. 85

5. The method of making low carbon alloys of iron, chromium and titanium, which consists in charging into an electric furnace a mixture of ferro-chromium high in carbon and a sufficient quantity of rutile to 90 decarbonize the alloy.

6. The method of making low carbon alloys of iron, chromium and titanium, which consists in charging into an electric furnace a mixture of ferro-chromium high in 95 carbon, a sufficient quantity of titanic oxid to decarbonize the alloy, and a sufficient quantity of burnt lime to form a protective slag.

In testimony whereof I have hereunto signed my name.

HUGH C. SICARD.